

No. 675,455.

Patented June 4, 1901.

J. B. TIBBITS, Dec'd.

LE GRAND C. TIBBITS, Administrator.

PROCESS OF MANUFACTURING LEAD SALTS BY ELECTROLYSIS.

(Application filed Mar. 6, 1894.)



FIG. 1.



FIG. 5.



FIG. 2.



FIG. 3.



FIG. 4.

WITNESSES:

Wm. Wilcox.  
Charles H. Knighton.

INVENTOR:

JOHN B. TIBBITS.

By Franklin Scott, Attorney.

# UNITED STATES PATENT OFFICE.

JOHN BLEECKER TIBBITS, OF HOOSICK, NEW YORK; LE GRAND C. TIBBITS  
ADMINISTRATOR OF SAID JOHN BLEECKER TIBBITS, DECEASED.

## PROCESS OF MANUFACTURING LEAD SALTS BY ELECTROLYSIS.

SPECIFICATION forming part of Letters Patent No. 675,455, dated June 4, 1901.

Application filed March 6, 1894. Serial No. 502,570. (No specimens.)

*To all whom it may concern:*

Be it known that I, JOHN BLEECKER TIBBITS, of the town of Hoosick, in the county of Rensselaer and State of New York, have  
5 invented certain Improvements in the Art of  
Manufacturing Lead Salts by Electrolysis,  
which invention is an improvement upon the  
invention set forth in Letters Patent of the  
United States of America No. 414,935, issued  
10 November 12, 1889, to Turner D. Bottome,  
which Letters Patent are now owned by me;  
and I hereby declare that the subjoined de-  
scription of the process for carrying out said  
invention and of the best method of working  
15 the same constitutes a specification thereof.

The object of the present invention is to  
obtain colored pigments having lead as bases  
by electrolytic action.

In the specification of the Letters Patent  
20 above cited a process for manufacturing  
white lead by electrolysis of a solution with  
leaden anodes is described. According to  
the present invention I modify said process  
so as to produce shaded or colored hydrated  
25 carbonate of lead.

For the purpose of best illustrating and ex-  
plaining the process which constitutes the  
subject-matter of this invention I have shown  
30 a simple apparatus in the accompanying  
drawings which is adapted to carry out the  
process constituting my invention.

Similar letters in said drawings indicate  
corresponding parts.

Figure 1 is a vertical section of the precipi-  
35 tating-tank, taken transversely to the plates  
which form the electrodes. Fig. 2 is a face  
view of one of the electrodes. Fig. 3 is an  
edge view of the same. Fig. 4 is a plan of  
the gas-distributing tubes, and Fig. 5 is an  
40 end elevation of the same.

To carry out this invention, a vat or tank  
E, which will not be affected by electrolytic  
action, is provided to hold the electrolytic sol-  
45 ution and to receive the precipitate. This  
solution is preferably alkaline. A system  
of tubing for introducing into and diffusing  
through this solution carbon dioxid is shown  
50 in Figs. 1, 4, and 5, which consists of a piece  
of rubber or glass tubing A, which is bent  
substantially to the shape shown, that por-  
tion which traverses the tank beneath the

electrodes being provided with lateral arms  
A', which have small perforations or diffusing-  
apertures A<sup>2</sup>, opening downwardly thereout,  
so as to effect a uniform diffusion of the gas 55  
through the bath. The bars F F span the top  
of the tank, and from them the electrodes B  
and C are suspended, being disposed in alter-  
nation. In the illustrations the anodes are  
represented by the compound plates B B B 60  
and the cathodes by the single plates C C C C.  
The body of the anode may be a plate of lead  
G, upon which are superposed copper strips  
D D D D. These attached metallic strips are  
termed "supplemental anodes." This com- 65  
bination and relative disposition of material  
in the exercise of the process will produce a  
precipitate of a brilliant blue tint, the same  
consisting chiefly of carbonate of lead and  
carbonate of copper. The apparatus is ren- 70  
dered effective by connecting all the anodes  
with each other and with the positive pole of  
the battery, and the cathodes are similarly  
connected with each other and with the nega-  
tive pole of the battery. The gas-distribut- 75  
ing pipe A is then connected with the source  
of supply of the carbon dioxid by one or both  
of its terminals, and enough pressure is ap-  
plied to the entering column of gas to effect  
its circulation through the bath. To procure 80  
a colored precipitate of which the lead shall  
form the base, I join with the lead of the elec-  
trode another substance, which in the proc-  
ess of the electrolytic decomposition of said  
substance and of the lead of the anode and 85  
its attendant reactions will impart a distinct-  
ive color to the resultant precipitate.

The following illustrates the operation of  
my invention: To produce a blue pigment hav-  
ing a lead base, I prepare an electrode (the 90  
anode) by attaching a piece of copper to a  
lead plate, so that they shall be in contact,  
and immerse this composite electrode in the  
electrolytic solution, so that both metals shall  
be in contact with the solution. The other 95  
electrode (or cathode) may be simply a plate  
of lead similarly immersed. Connection with  
the current is then made in the usual way,  
taking care, however, that the wire or other  
connection with the composite electrode is 100  
made with the element offering the highest  
resistance to the current, which in this in-

stance is the lead. The path of the current is thus from the lead of the positive side of the battery, through the copper, with which it must be in contact, into and through the bath, 5 to the cathode. In its passage such a reaction is set up that a blue product is precipitated as a result of the electrolytic action, which may be recovered from the bath and after being washed is found to be a true metallic pigment of great body and purity of color, the same consisting chiefly of carbonate of lead and copper. The depth of tone or intensity of color of the product is determined by the relative areas of the lead and 10 copper of the anode, the smaller the relative area of the copper used in comparison with that of the lead the lighter the tint.

A beautiful purple pigment can be obtained by coating all of the plates of the battery, both anode and cathode, with a strong solution of iodin well dried on. Then place them in the electrolytic solution, to which has been previously added a sufficient quantity of anilin-red or other suitable dye, which may 20 be poured into said solution in liquid form or dropped thereon as a powder and stirred in. Then connect with the current, when the product will be precipitated, which will be of a strong purple or violet color, which may be 25 recovered and washed, as described in the Letters Patent before recited.

Besides iodin, above mentioned, any mineral substance may be substituted for the cop-

per if of a nature to produce a colored pigment when subjected to electrolytic action, 35 as described. I am unable to name all such substances or to state the reactions. These last will differ with different substances.

By the word "composite" as used in this specification I mean composed of more than 40 one material. By the words "pigment coloring" as used in this specification I mean adapted to give color to what would otherwise be a white pigment when subjected to electrolysis in the conditions stated. 45

I therefore claim as my invention the following:

1. A process of manufacturing colored pigments consisting in electrolytically dissolving in an alkaline solution an electrode consisting of lead and another substance capable of imparting a color to lead salts, and supplying carbon dioxid to the bath. 50

2. A process of manufacturing colored pigments consisting in electrolytically dissolving in an alkaline solution, an electrode consisting of lead and copper and supplying carbon dioxid to the bath. 55

In witness whereof I have hereto subscribed my name this 28th day of February, A. D. 60 1894.

JOHN BLEECKER TIBBITS.

In presence of—

GEORGE H. MYERS,  
FRANKLIN SCOTT.